

Patented Jan. 13, 1931

1,788,876

# UNITED STATES PATENT OFFICE

DAVID LAMON, OF DENVER, COLORADO

## METAL TREATING COMPOSITION

No Drawing.

Application filed March 1, 1930. Serial No. 432,561.

My present invention relates to an improved metal treating composition of the molybdc class, for hardening and strengthening such metals as iron, steel, copper, and their alloys.

The different metals and their alloys may be treated with my composition for enhancing their commercial value, widening their scope of usefulness, and increasing their physical properties, without in any way impairing any of their properties of value which are previously possessed.

Thus the softer forms of iron, steel, and their alloys, when treated with my improved composition, have imparted thereto a fine grain, which is retained when the treated metal is subsequently subjected to thermal, mechanical treatment, in the formation of tools, structures, and other commercially useful articles. The improved steel is particularly adapted to and useful in the manufacture of gear wheels, high speed tool steel and in other devices where toughness, rigidity, strength and hardness are necessary requisites.

Brass and copper may also be treated by my improved composition, and after the copper has been treated according to my invention, the metal has imparted thereto a considerable degree of elasticity, and its tensile strength is enhanced, without materially impairing or lowering its ductility. Such treated metal is especially advantageous for use in strips and wires, such as are employed as electrical conductors, and for electric resistance devices.

The improved composition is comprised of the following ingredients:—boric acid, cyanide of potassium and molybdenum in proper portions, and the composition is varied as to quantity used according to different existing conditions.

From the molybdenum, which is obtained in crystalline crusts, molybdates or salts are derived, and acid molybdc is also derived.

For general use, the following formula may be followed:

|                                  | Parts |
|----------------------------------|-------|
| Cyanide of potassium             | 2     |
| Boric acid                       | 1 50  |
| Acid molybdc (50 to 85 per cent) | 1     |

In some instances, to the preceding formula is added the use of acid molybdc anhydride 100%, one half of a part.

Another formula contains:

|                                  | Parts |
|----------------------------------|-------|
| Boric acid                       | 1     |
| Potassium cyanide                | 2     |
| Acid molybdc (50% to 85%) C P    | 4     |
| Acid molybdenum anhydride (100%) | 1 60  |

In preparing them for use the ingredients are thoroughly pulverized and mixed to form the compound or composition, ready for use.

In the treatment of the metal with the composition, the steps of the following process are carried out. The metal or alloy to be treated (or the metal in a manufactured form) is heated in a furnace, either of intermittent or continuous operation, and by impingement of a non-luminous flame, is brought to a semi-molten state, after which the surface of the heated metal is sprinkled or covered with the composition or compound.

The proportions of the ingredients of the compound may vary, and the degree of temperature to which the treated metal is subjected may also vary in accordance with the nature of the metal. In the treatment of copper, the approximate temperature may be 600 degrees F.; for brass 700 to 1000 degrees F.; and for iron or steel, the temperature may vary between approximately 1200 to 1900 degrees F. The temperature is maintained for a suitable period of time during which the chemical action of the composition on the treated metal hardens, toughens, and strengthens the metal to a desired degree, without the necessity for use of an alloy.

The processed metal is then cleaned and allowed to gradually cool.

In some instances the processed molten metal is passed through a water solution of citric acid, with a salt of copper, such as a sulphate.

Having thus fully described my invention, what I claim as new and desire to secure by Letters Patent is:—

10 1. An improved composition for the treatment of metal comprising:

|                      | Parts |
|----------------------|-------|
| Cyanide of potassium | 2     |
| Boric acid           | 1     |
| Acid molybdic        | 1     |

15 2. An improved composition for the treatment of metals comprising:

|                         | Parts |
|-------------------------|-------|
| Cyanide of potassium    | 2     |
| Boric acid              | 1     |
| Acid molybdic           | 1     |
| Acid molybdic anhydride | ½     |

20 3. An improved composition for the treatment of metals comprising:

|                                  | Parts |
|----------------------------------|-------|
| Boric acid                       | 1     |
| Potassium cyanide                | 2     |
| Acid molybdic (50% to 85%) C P   | 4     |
| Acid molybdenum anhydride (100%) | 1     |

25 30 In testimony whereof I have affixed my signature.

DAVID LAMON.

35

40

45

50

55

60

65